

## UNITED STATES PATENT OFFICE

2,515,691

## AZO DYESTUFFS AS PHOTOGRAPHIC COUPLING COMPONENTS

Jules Edmond Beersmans, Bergerhout-Antwerp, Belgium, assignor to Gevaert Photo-Producten N. V., Martsel-Antwerp, Belgium, a company of Belgium

No Drawing. Application August 15, 1947, Serial No. 768,936. In Great Britain August 21, 1946

8 Claims. (Cl. 95-6)

1

The present invention relates to the production of color photographic images for color photography and more particularly to dyestuff intermediates for use in color photographic processes, especially by the process known as color development.

It is known that a colored photographic image may be formed simultaneously with the development of a silver image in an exposed photographic silver halide emulsion layer if an aromatic developing agent is used in the presence of a color coupler which couples with the oxidation product of such developer produced during development to form quinone-imine or azomethine dyestuffs.

The formation of azomethine dyestuffs necessitates the presence of a color coupler which contains a reactive methylene group linked on both sides with an electro-negative group. The most commonly used electro-negative groups known from the literature are  $-\text{CN}$ ,  $-\text{CO}-$ ,  $-\text{CS}-$ , nitrophenyl, the residue of a nitrogen containing five- or six-membered heterocyclic ring or a carbimide group  $=\text{C}=\text{N}-$  as in a pyrazolone nucleus.

Many such color couplers have been described in the literature, but the requirements for a satisfactory color coupler are rather strict. If it is to be incorporated in a photographic emulsion layer in the course of manufacture it should not have any deleterious influence upon the sensitizers or stabilizers of the emulsion and neither the coupler itself nor the dyestuff derived from same should have any substantial tendency to diffuse from such layer either into adjacent layers of the photographic element or into processing baths. If the coupler is to be added to the developer, there are still many requirements which must be met; thus it must not produce color fog on development, it must be stable to the alkaline substances of the developing bath which in turn must be stable to the oxygen of the air and so on. The number of the couplers known does not yet suffice to allow a free choice in view of the required shade and intensity of the dyestuff formed on development while furthermore the possibility of producing the coupler at an economic price must be taken into consideration.

It is an object of the present invention to provide a new process for developing a reducible silver salt image in a photographic element by means of a developing agent in the presence of a color coupler.

Another object of the present invention is to provide a photographic material containing a new color coupler.

A further object of the present invention is to provide a photographic developer containing a new color coupler.

2

Further objects will appear from the following description:

According to the present invention a valuable new class of "color couplers" is offered for the production of color photographic images by color development, which couplers contain a reactive methylene group linked on both sides to an electro-negative group, one of which is an azo group. These couplers may correspond to one or other of the following probable general isomeric formulae:



wherein

15  $\text{X}$ =either any activating group e. g.  $-\text{CN}$ ,  $-\text{CO}-$ ,  $-\text{NO}_2$  or a  $-\text{CHOH}-$  group,  
 $\text{R}=\text{H}$ , a carboxylic group, halogen, an azo- or hydrazone grouping or other easily removable atom or grouping,

20  $\text{R}'=\text{aryl}$  or a heterocyclic ring, either substituted or not.

In the following description, use will be made of only one form of the above given isomeric formulae but it is to be understood that the named compounds may be constituted according to the other form.

Examples of particular compounds of use in the present invention are:

30 1. Phenylazo acetone



2. alpha phenylazo acetyl acetic acid



35 3. phenylazo cyano acetic acid



40 4. phenylazo acetonitrile



45 5. phenyl azo-nitro-methane



60 6. p-nitro-phenyl azo-cyano acetic acid



55 7. alpha-naphthyl azo-cyano acetic acid



60

## 3

8. p-phenyl azo-phenyl azo acetonitrile.



9. diphenylene-p-p'-bis(azo acetonitrile)



10. bis(phenylazo) acetonitrile



Compounds which contain the group:



are for instance hydrazones of aldoses:

Lactose-phenyl-hydrazone,  
 Maltose-phenyl-hydrazone,  
 L-Arabinose-phenyl-hydrazone,  
 D-Glucose-p-tolyl-hydrazone,  
 D-Glucose-2:5-dichloro-phenyl-hydrazone,  
 L-Arabinose-p-bromo-phenyl-hydrazone.

The new color formers may be prepared by any convenient method.

Phenylazocetone may be prepared by reaction between acetylacetic acid and a diazobenzene chloride (JAPP. Ann 247,217). Alpha-phenyl-azo-acetic acid is first formed in this reaction.

Phenyl azo cyanacetic acid may be obtained by saponifying phenyl azocyanacetic acid ester by boiling for one hour in a 4% solution of NaOH in a mixture of equal proportions of alcohol and water. The product melts at 157° C. It may be decarboxylated by prolonged boiling to form phenyl azo acetonitrile. (cf. Bertini Gaz. Chem. Ital. 31 I 579).

Phenyl azo nitro methane may be obtained by allowing to react isonitromethane and diazo benzene (Bamberger, Berichte 33, (1900) 2060 and 34 (1901) 580).

p-Nitro phenyl azo cyan acetic acid may be obtained by heating the corresponding ester (prepared according to Ullman J. pr. Chem. 2, 51 (1895) 218) with 30 cc. NaOH 2 N and 30 cc. alcohol for one hour. The precipitate formed is sucked off and washed with alcohol. The sodium salt of the desired compound is obtained.

Bis(phenyl azo) acetonitrile may be obtained by allowing to react 2 mol. diazo-benzene and 1 mol cyanacetic acid according to Weissbach J. pr. Chem. 2 67 400 or Wedekind Ber. 30 2995.

According to the substituents in the molecule of the color couplers and to the developing agent chosen, yellow, magenta, or cyan dyestuffs having widely varying shades are obtained on color development. The new color couplers may be included either in the developing solution or added to a silver halide emulsion layer in the course of manufacture, or in a water-permeable colloid layer coated next to a silver halide emulsion layer or separated therefrom only by a thin water-permeable layer. When they are incorporated in a photographic layer, it is often advantageous to introduce in their molecule substituents rendering same diffusion-fast such as chains of more than five C atoms, biphenyl-groups or the like.

## Example 1

An exposed silver halide emulsion layer is developed in a bath of the following composition:

## 4

## A

|   |                                               |                  |      |
|---|-----------------------------------------------|------------------|------|
| 5 | N:N-diethyl-p-phenylene diamine hydrochloride | gm               | 2    |
|   | Sodium sulphite (crystals)                    | gm               | 25   |
|   | Sodium carbonate (crystals)                   | gm               | 60   |
|   | Sodium hydroxide                              | gm               | 2    |
|   | Water to                                      | cm. <sup>3</sup> | 1000 |

## B

|    |                           |                  |    |
|----|---------------------------|------------------|----|
| 10 | Phenylazo cyanacetic acid | gm               | 3  |
|    | Methyl alcohol            | cm. <sup>3</sup> | 30 |

For use, B is added to A.

After fixing and eliminating the reduced silver, a transparent magenta dyestuff image is obtained.

## Example 2

An exposed silver halide emulsion is developed in a bath containing the following substances:

|    |                                               |                  |      |
|----|-----------------------------------------------|------------------|------|
| 20 | A                                             |                  |      |
|    | N:N-diethyl-p-phenylene diamine hydrochloride | gm               | 2    |
|    | Sodium sulphite (crystals)                    | gm               | 25   |
|    | Sodium carbonate (crystals)                   | gm               | 60   |
| 25 | Sodium hydroxide                              | gm               | 2    |
|    | Water to                                      | cm. <sup>3</sup> | 1000 |

## B

|    |                          |                  |    |
|----|--------------------------|------------------|----|
| 30 | Glucose phenyl hydrazone | gm               | 3  |
|    | Methyl alcohol           | cm. <sup>3</sup> | 30 |

For use, B is added to A.

After fixing and eliminating the reduced silver, a transparent magenta dyestuff image is obtained.

## Example 3

An exposed silver halide emulsion layer is developed in a bath of the following compositions:

|    |                                               |                  |      |
|----|-----------------------------------------------|------------------|------|
| 40 | A                                             |                  |      |
|    | N:N-diethyl-p-phenylene diamine hydrochloride | gm               | 2    |
|    | Sodium sulphite (crystals)                    | gm               | 25   |
|    | Sodium carbonate (crystals)                   | gm               | 60   |
| 45 | Sodium hydroxide                              | gm               | 2    |
|    | Water to                                      | cm. <sup>3</sup> | 1000 |

## B

|    |                         |                  |    |
|----|-------------------------|------------------|----|
| 50 | Phenylazo nitro-methane | gm               | 3  |
|    | Methyl alcohol          | cm. <sup>3</sup> | 30 |

For use, B is added to A.

After fixing and eliminating the reduced silver, a transparent magenta dyestuff image is obtained.

## Example 4

An exposed silver halide emulsion layer is developed in a bath of the following composition:

|    |                                               |                  |      |
|----|-----------------------------------------------|------------------|------|
| 60 | A                                             |                  |      |
|    | N:N-diethyl-p-phenylene diamine hydrochloride | gm               | 2    |
|    | Sodium sulphite (crystals)                    | gm               | 25   |
|    | Sodium carbonate (crystals)                   | gm               | 60   |
|    | Sodium hydroxide                              | gm               | 2    |
|    | Water to                                      | cm. <sup>3</sup> | 1000 |

## B

|    |                                  |                  |    |
|----|----------------------------------|------------------|----|
| 65 | p-Nitrophenylazo cyanacetic acid | gm               | 3  |
|    | Methyl alcohol                   | cm. <sup>3</sup> | 30 |

For use, B is added to A.

After fixing and eliminating the reduced silver, a transparent blue dyestuff image is obtained.

## Example 5

An exposed silver halide emulsion layer is developed in a bath of the following composition:

|                             |                  |      |
|-----------------------------|------------------|------|
| Hydroquinone                | gm.              | 5    |
| Sodium sulphite (crystals)  | gm.              | 5    |
| Sodium carbonate (crystals) | gm.              | 60   |
| Water to                    | cm. <sup>3</sup> | 1000 |

|                              |                  |    |
|------------------------------|------------------|----|
| Phenylazo cyanacetic acid    | gm.              | 2  |
| Sodium carbonate 25 per cent | cm. <sup>3</sup> | 20 |
| Ethyl-alcohol                | cm. <sup>3</sup> | 30 |

group, nitrophenyl, a residue of a nitrogen-containing heterocyclic ring having a free bond in the 2-position with respect to the nitrogen atom, such residue having a free bond in the 4-position, a carbimide group ( $\text{---C}=\text{N}$ ), a nitro group and a  $\text{---CHOH}$  group, the hydrazone isomers of said compounds, and said compounds and isomers wherein a H-atom of the reactive methylene group is replaced by a grouping which is easily eliminated and selected from the class consisting of a halogen, a carboxylic group and an azo group.

5. Photographic developer comprising an aromatic developing agent for a latent silver halide image and a color coupler capable of coupling with the development product of said developing agent and selected from the class consisting of compounds containing a reactive methylene group immediately linked to an azo group and to a group selected from the class consisting of a cyan group, a carbonyl group, a thiocarbonyl group, nitrophenyl, a residue of a nitrogen-containing heterocyclic ring having a free bond in the 2-position with respect to the nitrogen atom, such residue having a free bond in the 4-position, a carbimide group ( $\text{---C}=\text{N}$ ), a nitro group and a  $\text{---CHOH}$  group, the hydrazone isomers of said compounds, and said compounds and isomers wherein a H-atom of the reactive methylene group is replaced by a grouping which is easily eliminated and selected from the class consisting of a halogen, a carboxylic group and an azo group.

6. Photographic developer comprising an aromatic developing agent for a latent silver halide image and a color coupler capable of coupling with the development product of said developing agent and corresponding to one of the following isomeric formulae

40 CN—CH<sub>2</sub>—N=N—aryl and CN—CH=N—NH—aryl

7. Photographic developer comprising an aromatic developing agent for a latent silver halide image and an aldose aryl hydrazone.

45 8. Photographic developer comprising a developing agent for a latent silver halide image and a color coupler capable of coupling with the development product of said developing agent and corresponding to one of the following isomeric formulae



55 and



JULES EDMOND BEERSMANS.

#### REFERENCES CITED

The following references are of record in the file of this patent:

#### UNITED STATES PATENTS

| Number       | Name          | Date          |
|--------------|---------------|---------------|
| 2,434,272    | Jelley et al. | Jan. 13, 1948 |
| 2,435,616    | Vittum et al. | Feb. 10, 1948 |
| 2,453,661    | Glass et al.  | Nov. 9, 1948  |
| 70 2,455,169 | Glass et al.  | Nov. 30, 1948 |
| 2,455,170    | Glass et al.  | Nov. 30, 1948 |

#### FOREIGN PATENTS

| Number     | Country       | Date          |
|------------|---------------|---------------|
| 75 503,824 | Great Britain | Apr. 11, 1939 |